

## UNITED STATES PATENT OFFICE

1,970,469

## MANUFACTURE OF RUBBER

Edward Arthur Murphy, Erdington, Birmingham, England, assignor to Dunlop Rubber Company, Limited, Erdington, Birmingham, England, a British corporation

No Drawing. Application December 15, 1933, Serial No. 702,563. In Great Britain November 23, 1932

4 Claims. (Cl. 106—23)

This invention comprises improvements in or relating to the manufacture of rubber compositions, and is particularly concerned with the production from aqueous dispersions of the kinds 5 hereinafter specified of powder-like compositions containing rubber or the like.

The present invention is a modification or development of the inventions set forth in Patent 1,953,972 and in pending applications, Serial No. 10 592,437, filed February 11, 1932, and Serial No. 610,496, filed May 10, 1932. The main modification or development consists in the step of converting the products obtained after removing all or most of the aqueous medium into a powder.

15 According to my invention, the process for the production of powder-like compositions containing rubber from aqueous dispersions of rubber or the like of the kinds hereinafter specified comprises effecting coagulation of the aqueous dispersions aforesaid in any of the manners set forth in the above applications, removing all or most of the aqueous medium so as to obtain a substantially dry product and converting or crumbling the dried product into a powder.

20 25 If desired, the aqueous medium can be removed by a filtration operation followed by a drying operation.

The powder-like compositions produced according to the present invention can be very efficiently used in the production of moulded articles. In many cases, a cold moulding operation without subsequent heating or vulcanization is sufficient.

30 35 The powder-like compositions produced according to the present invention can be admixed with granular, fibrous or divided materials such as leather fibre, wood flour, cork dust, jute fibre, cotton flock, paper pulp, naturally short cellulose fibres and ground fibres or alternatively or additionally with mineral powders such as whiting or sand, either by admixing these materials direct with the powder-like compositions or by admixing these additional materials with the intermediate flocculent or granular precipitates and thereafter 40 45 removing all or most of the aqueous medium and converting or crumbling the substantially dried product into a powder.

50 These powders are also capable of being pressed up cold to give hard moulded products. The products obtained according to the present invention are of particular use for moulding operations in view of the shortness of the mould cycle and the ability to use bright colours. The ability to produce coherent masses merely by cold moulding appears to be associated with a characteristic

adhesiveness frequently observed in connection with flocculent or granular precipitates.

The method of effecting coagulation of the aqueous dispersions aforesaid in the presence of a relatively large quantity of water as set forth 60 in application Serial No. 592,437 by precipitating in situ one or more compounding ingredients preferably in relatively large proportions on the rubber content by the interaction or double decomposition of one or more water soluble reagents having normally no coagulating effects upon the aforesaid dispersions with one or more water soluble reagents subsequently added thereto is of particular use in connection with the 65 present invention.

70 Examples of the water soluble reagents of the first class having normally no coagulating effects upon the dispersions are—carbonates, sulphates, silicates of the alkali metals or of ammonium.

75 Examples of the water soluble reagents of the second class which interact with the water soluble reagents of the first class to produce insoluble compounding ingredients are soluble salts of magnesium, aluminium, calcium, barium or zinc; sodium silicate also falls into this class if the 80 corresponding reagent in the first class is such as to precipitate silicic acid—e. g. ammonium carbonate.

85 By a suitable choice of the reagents and consequent reaction products precipitates of varying consistency can be formed.

If desired, the granular precipitates can be washed free from soluble reaction products such as soluble sulphates or chlorides by known means such as filtration and washing prior to their consolidation or concentration.

90 Numerous substances are capable of being used as compounding ingredients, for example, carbonates of magnesium, calcium and zinc may be prepared from sodium carbonate and sulphates or chlorides of these metals. Similarly the silicates of magnesium and zinc can be prepared from sodium silicate and the corresponding sulphate or chloride.

95 100 Mixtures of precipitates may be prepared and the reactions may be chosen in such a manner that only one soluble reaction product results for two insoluble products, for example, the reaction between one equivalent of sodium carbonate and one of magnesium sulphate followed by one equivalent of barium chloride yields only one equivalent of sodium chloride for two equivalents of mixed precipitate.

105 110 In this manner, a larger yield of precipitate

may be obtained relative to the amount of soluble salt formed.

The reagents may be added in the form of their aqueous solutions and may contain protective colloids such as glue, gum acacia, in solution to increase the fineness of subdivision of the precipitated compounding ingredients.

The rate at which coagulation takes place after the introduction of the water soluble reagents of the second class may be controlled by the addition of suitable substances, for example, casein.

Other examples of suitable coagulants are acetic acid, salts such as zinc sulphate and magnesium sulphate.

The emulsions or dispersions of rubber or the like comprise those consisting of rubber, gutta-percha, balata or similar vegetable resins occurring naturally or artificially obtained. Such artificial aqueous dispersions may include those of coagulated rubber, vulcanized rubber, synthetic rubber, waste or reclaim.

If desired, any of the aforementioned dispersions may be used alone or in admixture with one another. Any of the aforesaid dispersions may contain the usual known compounding and vulcanizing ingredients and/or may be in concentrated form.

Concentrates such as are obtained in Patent 1,846,164, February 23, 1932, or in British Patent 219,635 to which may be added any one or more of the usual compounding ingredients may also be used.

The aforesaid vulcanizing and other compounding ingredients which are added in the form of their dispersions may be added to the aforesaid aqueous emulsions or dispersions of rubber or the like prior or subsequent to the precipitation of the granular dispersions.

It is preferable to add the aforesaid dispersions of the vulcanizing and other compounding ingredients before the precipitation of the granular dispersions.

In some cases, where the precipitate obtained is found to be in a damp powdery or short paste-like condition before consolidation into the compact uniform mass, consolidation can be hastened and facilitated by treating the filter cake obtained with a rubber solvent which may be mixed with a mutual solvent for the water and the rubber solvent employed, as for instance alcohol.

The following examples illustrate how the process can be effected.

#### Example 1

An unvulcanized rubber powder having for example the following suitable composition—

|                    | Parts by weight |
|--------------------|-----------------|
| Rubber             | 60              |
| Aluminium silicate | 40              |

can be produced as follows—

100 parts of concentrated latex of 60% concentration produced by centrifugalization is diluted to a 5% concentration. 104 parts of 50% sodium silicate in the form of a 5% solution are stirred into the latex and this is followed by the addition of 96 parts of aluminium sulphate also in the form of a 5% solution. The precipitate so formed is filtered, dried and disintegrated into a powder.

The rubber powder so produced can be formed into a sheet by pressing it up in a cold mould.

If desired, the dry uncompounded rubber powder can be mixed with compounding ingredients

to form a composition for direct moulding purposes.

#### Example 2

The flocculent precipitate produced in accordance with Example 1 can be mixed with granite chippings, the admixture allowed to dry and then coarsely disintegrated. The coated chippings may be consolidated into a more or less uniform sheet by cold pressure such as rolling producing in this way rubber products for surfacing roads and other structures.

#### Example 3

A flocculent granular precipitate of the following composition—

|                    | Parts by weight |
|--------------------|-----------------|
| Rubber             | 100             |
| Sulphur            | 5               |
| Zinc oxide         | 5               |
| Accelerator        | 0.5             |
| Aluminium silicate | 15              |

is first prepared as follows—

To 340 parts by weight of a 60% rubber latex obtained by centrifugal action, the following ingredients are added with constant stirring and in the following order—

- (1) 20 parts by weight of a 50% sulphur dispersion.
- (2) 20 parts by weight of a zinc oxide 50% dispersion.
- (3) 2.8 parts by weight of a 35% accelerator dispersion.
- (4) 1840 parts by weight of water plus 78 parts by weight of a 5% sodium silicate solution.
- (5) 650 parts by weight of water plus 72 parts by weight of aluminium sulphate crystals.

In this way, a rubber precipitate is obtained wherein the concentration of the precipitate in the aqueous medium is 5%.

The resulting rubber precipitate is allowed to drain on a filter and a paste-like mass is obtained containing approximately 18% total solids.

This paste-like mass is compounded with disintegrated leather dust in the proportion to give 70 parts of leather dust to 30 parts of dry precipitate. The admixture is then dried and finally disintegrated.

The disintegrated powder-like crumb can be put into a mould and pressed up cold for 30-40 seconds under a pressure of 5000 lbs., per square inch to produce a hard leather-like moulded article.

#### Example 4

The paste-like mass prepared according to Example 3 can be mixed with sand and slate flour in the proportion of 10 parts of rubber precipitate, calculated on the dry weight, 60 parts sand and 30 parts slate flour. This admixture is dried and disintegrated.

This powder can be cold moulded under pressure to give a hard wood-like product. Using suitable compounding ingredients highly coloured horn-like materials can be made in this way.

Whereas heretofore the flocculent precipitates when dry have been consolidated only by the use of heat and pressure, the present invention provides a powdered rubber composition with sufficient cohesiveness so that the powder-like particles can be consolidated into a solid mass by the use of pressure and at ordinary temperatures. This enables the material to be used with colors that could not be used where high temperatures

are involved and also makes the moulding operation much easier and simpler.

Having now particularly described my invention, I claim—

- 5 1. A method for the manufacture of cold moldable powders comprising rubber material which comprises forming a washable crumb-like suspension of said material from an aqueous dispersion thereof by adding to said dispersion a water soluble reagent having normally no coagulative effect upon the dispersion, then adding a reagent to form a water insoluble inert inorganic compounding ingredient by interaction with said first reagent and simultaneously coagulating said 10 rubber dispersion to form a granular precipitate, drying said precipitate, and disintegrating the same to a powder.
- 15 2. The process of claim 1 in which said inorganic inert precipitate is a silicate.

20

EDWARD ARTHUR MURPHY.

25

30

35

40

45

50

55

60

65

70

75

3. The process of claim 1 in which said precipitates are admixed with fillers.

4. A method for the manufacture of cold molded articles comprising rubber material which comprises forming a washable crumb-like suspension of said material from an aqueous dispersion thereof by adding to said dispersion a water soluble reagent having normally no coagulative effect upon the dispersion, then adding a reagent to form a water insoluble inert inorganic compounding ingredient by interaction with said first reagent and simultaneously coagulating said rubber dispersion to form a granular precipitate, drying said precipitate, disintegrating the same to a powder, and compressing said powder without heating to a compact adherent mass.

80

85

90

95

100

105

110

115

120

125

130

135

140

145

150